

## UNITED STATES PATENT OFFICE

2,126,753

COMPOSITE FABRIC AND METHOD OF  
MAKING SAME

Camille Dreyfus, New York, N. Y.

No Drawing. Application August 4, 1934,  
Serial No. 738,429

6 Claims. (CL. 154—2)

This invention relates to the preparation of stiffened composite or laminated fabrics and also to wearing apparel or other technical or industrial articles formed in whole or in part of such 5 stiffened fabrics.

An object of my invention is to prepare fabrics of any desired degree of increased stiffness and in a simple and expeditious manner. A further object of my invention is to prepare wearing apparel or other technical or industrial articles consisting of or containing such stiffened fabric. Other objects of the invention will appear from the following detailed description.

I have found that stiffened fabrics may be prepared at low cost and very simply by pressing an assembly of fabrics made of or containing non-thermoplastic fibres, at least one layer of fabric, which will usually be an interposed layer, being coated or impregnated with cellulose acetate or 10 other organic derivative of cellulose in powdered or finely divided form. The assembly is subjected to pressing, at least locally, at elevated temperatures in the presence of a suitable liquid.

I have further found that by having present 15 volatile liquids, that are not active solvents for cellulose acetate at ordinary temperatures but which cause the same to stiffen at elevated temperatures, during the application of heat and pressure, many advantageous results are attained. Since these liquids are not active solvents at 20 ordinary temperatures, action on the cellulose acetate takes place only upon application of heat and pressure, and therefore by applying heat and pressure only locally, ornamental or other special 25 effects may be produced. The use of such non-solvents is preferred, since the use of liquids that are active solvents at ordinary temperatures is often disadvantageous. Such active solvents act too quickly and produce defects in the finished 30 article for various reasons, while with the use of non-solvents, such defects are avoided.

The products formed by my invention may be 35 used for any purpose where a stiffened and/or relatively impermeable fabric is desired. An important application of such products is wearing apparel, which wearing apparel may be formed in whole or in part of fabrics made or prepared 40 in accordance with this invention. Thus collars or cuffs may be formed entirely of the product of this invention. Alternatively shirts may be made wherein the attached collars, neckbands, cuffs, fronts or bosoms are made of such products. Hats or parts of hats may likewise be formed of 45 such material, as may also be the inner or sweat bands of hats, visors for caps, inner linings for 50

cravats, stiffening material used in the inner portions of garments, such as coats, to help retain the shape thereof, etc. The fabrics of this invention may be used for a variety of other purposes, and indeed may be used for any industrial 5 or technical purpose where fabric of increased stiffness and/or impermeability is required. Another use of the fabrics of this invention is in wrapping articles, in which case heat and pressure may be applied only locally to seal the pack- 10 age.

In one form of this invention the assembly of fabrics with an intermediate layer containing cellulose acetate in powder or finely divided form employed as starting material may first be cut, 15 sewn or otherwise shaped. After the desired articles, such as collars, cuffs or other wearing apparel or parts thereof, are formed, they may then be treated with a liquid that is either a solvent for the cellulose acetate or causes the cellulose 20 acetate to stiffen at elevated temperatures, and then subjected to heat and pressure to impart the desired stiffness and/or impermeability. In this manner the sewing of stiff material is avoided.

Products of this invention have any desired 25 degree of stiffness, which is relatively permanent, so that they may be subjected to repeated laundering without substantially losing their stiffness. In this manner the use of starch or other extraneous stiffening materials during laundering 30 may be avoided.

This invention may be carried out in a large 35 number of ways, having regard to the nature of the fabric or number of fabrics employed, provided that a layer of fabric comprising non-thermoplastic fibres and containing cellulose acetate in powder or finely divided form is interposed between a plurality of fabrics that consist of or contain non-thermoplastic fibres.

There should be present in the product treated 40 at least one layer of fabric consisting of non-thermoplastic fibres coated or impregnated with finely divided cellulose acetate and at least one layer, but preferably two or more layers, of fabric which consists wholly of non-thermoplastic 45 fibres such as cotton, linen, regenerated cellulose, wool or natural silks. Instead of employing fabrics consisting wholly of non-thermoplastic fabrics, any or all of the fabrics consisting wholly of non-thermoplastic fibres that do not contain 50 the finely divided or powdered cellulose acetate may be replaced by a mixed fabric containing yarn of cellulose acetate, alternating either in the warp or in the weft, or both, in any desired degree of alternation, with yarns of non-thermo-

plastic fibres. Instead of employing a woven fabric, a knitted or netted fabric containing the non-thermoplastic fibres may be employed.

In a method, in some cases preferred, of carrying out the invention, two or more fabrics consisting wholly of non-thermoplastic yarns, such as cotton, linen, reconstituted cellulose, wool or silk, are assembled with one or more interposed layers consisting of such non-thermoplastic yarns and containing cellulose acetate in powdered or finely divided form, and this assembly may be treated in accordance with this invention, whereby a composite fabric made up of a plurality of layers is produced. If a product is to be produced wherein all the layers thereof are united, it is of importance, where two or more layers of fabric consisting wholly of non-thermoplastic material are used, that at least one layer of fabric containing cellulose acetate in powdered or finely divided form be interposed between such layers of fabric.

In another form, two layers of fabric consisting of non-thermoplastic fibres may be coated with the finely divided cellulose acetate and assembled with the coated sides in juxtaposition, and this assembly then subjected to the uniting process.

As instances of the manner in which the various fabrics may be assembled, the following are given. In the case of collars, cuffs, etc. where an exterior of cotton or linen is desired, a layer of cotton fabric containing cellulose acetate in powdered or finely divided form, may be interposed between two layers of fabric consisting of cotton, linen or other non-thermoplastic fibres. An assembly that is also useful for such purposes comprises three layers of fabric consisting wholly of such non-thermoplastic yarns, with a layer of fabric of non-thermoplastic fibres containing cellulose acetate in powder form between each of such fabrics.

These arrangements are given only by way of example, it being obvious that other arrangements with a less or greater number of layers of fabric may be employed to obtain any desired effects.

Often, particularly in connection with wearing apparel or parts thereof, such as collars, cuffs, shirt bosoms, hats, etc., it is advantageous to cut or sew together the assembly to the desired form before subjecting the same to the stiffening operation, since it is much more convenient to manipulate them before the desired stiffness is imparted thereto.

The layer of fabric comprising non-thermoplastic fibres and containing cellulose acetate in powder form that may be used in carrying out this invention may be prepared in various manners.

In one mode of operation, fabrics of any desired construction and made of yarns of cotton, reconstituted cellulose, linen, natural silk, wool or other non-thermoplastic fibres may be impregnated with or coated with an aqueous or other suspension of very finely divided cellulose acetate, with or without plasticizer. If the water or other liquid used as the suspending mixture is permitted to evaporate substantially completely, the coated or impregnated fabric may be sold or shipped as a separate article of commerce and sale.

The cellulose acetate employed for this invention may be reduced to the finely divided form in any suitable manner. Thus it may be reduced to the size of an impalpable powder by prolonged grinding in a ball or pebble mill in the pres-

ence of water or other liquid used as a suspension medium. In another, and in some cases preferred, method the cellulose acetate and water or other suspension liquid is passed through a colloid mill provided with closely fitting rotors, one or both of which is provided with a carbonium or other abrasive surface, to form a slurry containing the finely divided cellulose acetate. If plasticizers are added, these will be present in very intimate admixture with the finely divided cellulose acetate.

In order to promote better adhesion of the finely divided cellulose acetate to the fabric, adhesives, binders or agglutinants, such for instance as gelatin, gum arabic, gum tragacanth or other gums, latex etc., may be incorporated with the finely divided cellulose acetate, and in many cases such adhesives, binders or agglutinants promote the adhesion of the treated fabric to the other fabrics with which it is laminated.

The suspension of the finely divided cellulose acetate may be applied to the fabric in any convenient manner as by means of a padding mangle, by passing the fabric through a bath of the suspension, with or without subsequent passage between quench rolls, by spraying or brushing the suspension of finely divided cellulose acetate onto the fabric, or in other ways.

Preferably the water or other suspending liquid is evaporated from the fabric after application of the suspension of cellulose acetate, and this may be done by passing the fabric through drying chambers or tenters, or around internally heated drums or cams.

In another mode of applying the cellulose acetate to the fabric, the cellulose acetate in the form of finely divided dry powder, with which a plasticizer may or may not be in intimate admixture, may be blown or sprayed onto fabrics comprising non-thermoplastic fibres and, if desired, gelatin, gums or other appropriate adhesives, agglutinants or binders may be employed to cause such powder to adhere to the fabric more readily.

To obtain good adhesion, an appropriate liquid should be present during the application of heat and pressure to the assembly of fabrics of non-thermoplastic fibres and the fabric containing finely divided cellulose acetate. Examples of such liquids are the active solvents for the cellulose acetate, such as acetone, ethyl lactate, formal glycerol, etc. The active solvents may be diluted with water or other liquids to restrict their solvent power. Solutions of plasticizers in volatile liquids that may or may not be active solvents may also be used for this purpose.

A preferred liquid to be used is a volatile liquid that acts on the cellulose acetate at elevated temperatures so as to cause the same to stiffen, but which is preferably not an active solvent at ordinary temperatures. I prefer to use for this purpose ethyl alcohol (denatured or undenatured) or methyl alcohol containing water, or mixtures of these, since they are relatively inexpensive. Ethyl alcohol containing about 20% of water is particularly desirable as its vapors are not toxic or disagreeable. Less advantageously, more or less water may be added to the alcohol. Aqueous solutions of ethyl alcohol or of methyl alcohol of 55 to 90%, particularly of about 80%, concentration are very useful for this purpose. Another example of a suitable liquid that may be used is an aqueous solution of the mono-methyl ether of ethylene glycol containing, say, about 20% of water. These liquids are not active

solvents for cellulose acetate at ordinary temperatures.

The liquid may be applied to the assembly of fabrics having an intermediate layer of fabric containing cellulose acetate in powdered or finely divided form in any suitable manner, such as by dipping, spraying or brushing. A convenient manner of wetting the assembly is by padding the same with the liquid. Both sides of the assembly should preferably be wetted with the liquid, as it is desirable that all of the layers of the fabric present be wetted therewith when heat and pressure is applied.

The so wetted assembly of fabrics is then subjected to heat and pressure. This may be done by any suitable device, for instance, by hot ironing or by passing between pressure rolls, one or both of which are heated, or between a heated roller and a heated or cold plate or surface, or between a heated pressing iron or plate and a cold board or surface. The heating device may be heated to the desired temperatures, for instance, 80 to 180° C. or more and the pressure applied may be any desired pressures, for instance, from 10 to 600 pounds per square inch.

If heated devices that have desired designs, such as stripes, dots, rectangles or other geometric, floral or other designs, embossed thereon are employed, novel effects are obtained, since only those portions that come in contact with the embossed portions of the heated device become united, while the other portions retain the properties of the original fabrics. This local application of heat and pressure may be done by manually operated means if desired.

In order further to illustrate my invention, but without being limited thereto, the following example is given.

*Example*

40 For making fabrics to be used for making any desired articles, there is employed an assembly of two layers of cotton or linen fabric with an interposed layer of cotton fabric coated or impregnated with acetone-soluble cellulose acetate in 45 finely divided or powder form.

To coat or impregnate the cotton fabric, a suspension is made of the following ingredients:

| Parts by weight    |      |
|--------------------|------|
| Cellulose acetate  | 100  |
| Dimethyl phthalate | 10   |
| Gum tragacanth     | 15   |
| Water              | 1000 |

This mixture is passed through a colloid mill 55 provided with carborundum rotors and is then further treated for one or two hours in a ball or pebble mill. The resulting suspension is then applied to a cotton fabric by means of a padding mangle after which the fabric is dried by passing 60 around drums or cams heated internally by steam.

The assembly of two layers of the cotton or linen fabric with the interposed layer of cotton fabric containing the finely divided cellulose acetate is then wetted on both sides with an aqueous solution of ethyl alcohol (denatured or not) of 65 20% concentration. Thereupon the assembly is pressed with a hot iron or calender to form a stiffened material in which the fabrics are 70 united. By controlling the degree of heat and pressure and/or selection of the type of fabrics employed and the amount of cellulose acetate present, the degree of stiffness may be controlled.

Generally a semi-stiff fabric is formed, which 75 retains its stiffness after repeated laundering so

that the use of starch or like material is not required.

If collars or cuffs or bosoms or other articles which are to be sewn onto shirts or other articles of apparel are to be formed, it is advantageous 5 to cut the assembly of fabrics to the desired shape or form and sew it to the shirt or other article prior to the application of the aqueous alcohol and the heat and pressure so that the assembly is stiffened and united by wetting with the 10 aqueous alcohol and application of heat and pressure only after the shirt or other article is completed.

The fabrics and articles obtained by this invention may be made more or less stiff as desired 15 by controlling the amount of finely divided cellulose acetate present in the assembly of fabrics being treated; the more cellulose acetate present, the stiffer the resultant products. The fabrics or other articles may be rendered softer by the 20 incorporation of more or less plasticizers, such as diethyl phthalate, dimethyl phthalate, dibutyl tartrate, etc., in the aqueous alcohol or onto or in the layer of fabric containing the cellulose acetate in finely divided form.

25 While this invention has been described particularly in connection with cellulose acetate, such cellulose acetate may be replaced in whole or in part by other derivatives of cellulose such as cellulose nitrate, or cellulose formate, cellulose propionate, cellulose butyrate, or other esters of cellulose, or methyl cellulose, ethyl cellulose and benzyl cellulose or other cellulose ethers, in which case suitable liquids having the required properties for aiding union under heat and pressure 35 will be selected.

It is to be understood that the foregoing detailed description is given merely by way of illustration and many variations may be made therein, without departing from the spirit of my 40 invention.

Having described my invention, what I desire to secure by Letters Patent is:

1. A method of preparing stiffened laminated fabric such as collars, cuffs and like articles of 45 wearing apparel, which comprises impregnating a fabric with a dispersion of finely divided thermoplastic derivative of cellulose in a non-solvent therefor, drying said impregnated fabric, assembling said impregnated fabric with at least one 50 other fabric, and forming a stiffened laminated fabric by subjecting the assembly of fabrics to heat and pressure in the presence of a liquid selected from the group consisting of aqueous solutions of methyl alcohol, ethyl alcohol and 55 monomethyl ether of ethylene glycol.

2. A method of preparing stiffened laminated fabric such as collars, cuffs and like articles of wearing apparel, which comprises impregnating a fabric with a dispersion of finely divided thermoplastic derivative of cellulose in a non-solvent therefor, said dispersion containing a binder, 60 drying said impregnated fabric, assembling said impregnated fabric with at least one other fabric, and forming a stiffened laminated fabric by 65 subjecting the assembly of fabrics to heat and pressure in the presence of a liquid selected from the group consisting of aqueous solutions of methyl alcohol, ethyl alcohol and monomethyl ether of ethylene glycol.

3. A method of preparing stiffened laminated fabric such as collars, cuffs and like articles of wearing apparel, which comprises impregnating a fabric with a dispersion of finely divided cellulose acetate in a non-solvent therefor, drying 70

said impregnated fabric, assembling said impregnated fabric with at least one other fabric, and forming a stiffened laminated fabric by subjecting the assembly of fabrics to heat and pressure in the presence of a liquid selected from the group consisting of aqueous solutions of methyl alcohol, ethyl alcohol and monomethyl ether of ethylene glycol.

4. A method of preparing stiffened laminated fabric such as collars, cuffs and like articles of wearing apparel, which comprises impregnating a fabric with a dispersion of 100 parts of finely divided cellulose acetate in 1000 parts of water containing 10 parts of dimethyl phthalate and 15 parts of gum tragacanth, drying said impregnated fabric, assembling said impregnated fabric with at least one other fabric, and forming a stiffened laminated fabric by subjecting the assembly of fabrics to heat and pressure in the presence of a liquid selected from the group consisting of aqueous solutions of methyl alcohol, ethyl alcohol and monomethyl ether of ethylene glycol.

5. A method of preparing stiffened laminated fabric such as collars, cuffs and like articles of wearing apparel, which comprises impregnating a fabric with a dispersion of finely divided thermoplastic derivative of cellulose in a non-solvent therefor, drying said impregnated fabric, assembling said impregnated fabric with at least one other fabric, and forming a stiffened laminated fabric by subjecting the assembly of fabrics to heat and pressure in the presence of aqueous alcohol. 5

6. A method of preparing stiffened laminated fabric such as collars, cuffs and like articles of wearing apparel, which comprises impregnating a fabric with a dispersion of finely divided cellulose acetate in a non-solvent therefor, drying said impregnated fabric, assembling said impregnated fabric with at least one other fabric, and forming a stiffened laminated fabric by subjecting the assembly of fabrics to heat and pressure in the presence of aqueous alcohol. 10 15

CAMILLE DREYFUS.